

## UNITED STATES PATENT OFFICE.

CLARENCE P. LINVILLE, OF ELIZABETH, NEW JERSEY, ASSIGNOR TO AMERICAN SMELTING AND REFINING COMPANY, OF NEW YORK, N. Y., A CORPORATION OF NEW JERSEY.

## ELECTROLYTIC TIN.

No Drawing.

Application filed December 30, 1920. Serial No. 434,118.

*To all whom it may concern:*

Be it known that I, CLARENCE P. LINVILLE, a citizen of the United States, and resident of Elizabeth, in the county of 5 Union and State of New Jersey, have invented certain new and useful Improvements in Electrolytic Tin, of which the following is a specification.

The invention relates in general to a certain new and useful improvement in the production of electrolytically refined tin from impure tin anodes and specifically relates to an additional agent for use in the electrolyte in the electrolytic refining of tin. The 15 invention constitutes an improvement in the process defined in the patent to R. L. Whitehead, No. 1,157,830, October 16, 1915 and constitutes a companion case with the applications of Harry H. Alexander, Serial 20 No. 434,124, and James Robert Stack, Serial No. 434,114, on Electrolytic refining of tin, filed under even date.

Heretofore, as disclosed in the said patent to Whitehead and as disclosed in the above identified applications, it is proposed to produce from impure tin which usually contains lead, and other impurities, an electrolyte of such character that it will insure the continued maintenance of electrolytic 30 decomposition of the tin during the refining operation. The Whitehead process consists fundamentally in maintaining at least a six percent solution of tin in the electrolyte and in this condition the process can be operated continuously when the electrolyte has in solution one-tenth of one per cent sulphuric acid and fifteen to twenty per cent of hydrofluosilicic acid. In the above identified Alexander application it is proposed to increase the sulphuric acid constituent and correspondingly decrease the hydrofluosilicic acid constituent to meet certain conditions defined in that application. With both of these hydrofluosilicic-sulphuric acid electrolytes it is found that under some conditions 45 polarizations would occur, the anodes would become insoluble presumably on account of the formation of hard slimes thereon and as a result the current would continue to plate 50 tin out and the electrolyte would quickly become depleted of tin. Further occasional out-growths are formed upon the cathodes causing short circuits with resulting low ef-

ficiency. These growths were particularly prevalent in those situations where too much additional agents were present at the temperature at which the process was practiced and it became a difficult problem to gauge the proper amount of additional agents which should be added to the electrolyte under the necessarily varying temperature conditions present.

Accordingly, one of the objects of the invention is to provide an improved form of hydrofluosilicic-sulphuric acid electrolyte having all of the virtues of this substance defined in the prior patent and applications, above identified, and which at the same time will defeat its tendency to form short circuiting sprouts or other polarizing action.

I attain this object broadly by incorporating in the electrolyte either a free halogen acid or a halogen salt capable of reacting with the electrolyte to form the acid. Hydrochloric acid (HCl) is suggested as suitable but this is only suggestive of one acid which has been found satisfactory under practical working conditions.

In a situation where there is an excess of sulphuric acid, sodium chloride (NaCl) or common salt may be added, in which case the reaction is presumably as follows:



In the case of the electrolyte defined in the above identified patent and applications it is found that the addition of two-tenths to three-tenths per cent of hydrochloric acid or its equivalent in the electrolyte gave the best results.

The presence of the sodium sulphate apparently has no effect upon the activity of the electrolyte and the addition of the salt has an economic value over the use of the hydrochloric acid in that the salt is cheaper. In the method defined in the Alexander application there is an ample excess of sulphuric acid to unite with the small amount of salt present to form the necessary amount of hydrochloric acid required by this process.

It is further suggested to add both the salt and the hydrochloric acid to the electrolyte containing sulphuric acid. The addition of the halogens eliminates the formation of hard slimes and thus maintains the solubil-

ity of the anode even in the presence of an excessive amount of addition agent and even when the electrolyte is heated. The anode corrosion is improved and a fine dense deposit is laid on the cathode.

Having thus described my invention, I claim:

1. An electrolyte for the deposition of tin free from lead, comprising an electrolytic solution of tin in hydrofluosilicic acid containing sulphuric acid in an amount sufficient to react with the lead present to form an insoluble lead salt and to provide an excess of free sulphuric acid and an agent capable of reacting with said excess of sulphuric acid to form free hydrochloric acid.
2. In the electrolytic refining of impure tin, the method of preventing contamination of the tin deposited from the impure tin 20 anode upon the cathode, which consists in employing as the electrolyte a solution of tin in hydrofluosilicic acid together with a quantity of sulphuric acid sufficient to convert the lead of the dissolving anode into lead sulphate and a substance having chlorine radical and capable of preventing polarization.
3. An electrolyte for the deposition of tin, free from lead, comprising an electrolytic solution of tin, said solution including hydrofluosilicic acid an agent to protect the

electrolyte from the lead present and a suitable soluble haloid salt.

4. An electrolyte for the deposition of tin, free from lead, comprising an electrolytic 25 solution of tin, said solution including hydrofluosilicic acid, and an agent to protect the electrolyte from the lead present, including sulphuric acid and a suitable soluble haloid salt.

5. An electrolyte containing tin in solution, sulphuric acid and a soluble haloid salt said solution including hydrofluosilicic acid.

6. An electrolyte containing tin in solution and free hydrochloric acid said solution including hydrofluosilicic acid.

7. An electrolytic solution comprising hydrofluosilicic acid having tin dissolved therein and including an agent to protect the solution from the action of any foreign material and including also a soluble haloid salt.

8. An electrolytic solution comprising hydrofluosilicic acid having tin dissolved therein and including sulphuric acid in an amount sufficient to react with any foreign material.

Signed at Perth Amboy in the county of Middlesex and State of New Jersey this 60 10th day of December, A. D. 1920.

CLARENCE P. LINVILLE.